

Aug. 21, 1928.

1,681,496

C. L. READ

PROCESS FOR REFINING CRUDE ARSENIC TRIOXIDE

Filed April 14, 1926

2 Sheets-Sheet 1



INVENTOR  
CHESTER L. READ  
BY  
albert M. Austin  
ATTORNEY

Aug. 21, 1928.

1,681,496

C. L. READ

PROCESS FOR REFINING CRUDE ARSENIC TRIOXIDE

Filed April 14, 1926

2 Sheets-Sheet 2



Fig. 4.



Fig. 5.

INVENTOR

CHESTER L. READ

BY *Albert M. Austin*

ATTORNEY

Patented Aug. 21, 1928.

1,681,496

# UNITED STATES PATENT OFFICE.

CHESTER L. READ, OF RAHWAY, NEW JERSEY, ASSIGNEE TO AMERICAN SMELTING AND REFINING COMPANY, OF NEW YORK, N. Y., A CORPORATION OF NEW JERSEY.

## PROCESS FOR REFINING CRUDE ARSENIC TRIOXIDE.

Application filed April 14, 1926. Serial No. 102,090.

The invention relates to a process for refining crude arsenic trioxide and particularly crude arsenic trioxide of high antimony content. According to the invention there may be produced from crude arsenic trioxide of high antimony content a high grade arsenic trioxide practically free from antimony, which is known to the trade as high grade white arsenic and which may contain not less than 99% pure arsenic trioxide and not more than 0.7% of antimony.

According to the invention crude arsenic trioxide commonly known as "black dust" which may be of high antimony content and which may contain other impurities, is treated in a refining furnace in a novel manner to produce pure high grade white arsenic. In the refining furnace the volume of air and the temperature particularly near the flue is controlled so that glassy arsenic trioxide or "vitreous arsenic" is deposited in the flue near the furnace. The remaining volatile crude arsenic trioxide passes over the vitreous arsenic which absorbs the antimony impurities therefrom so that the arsenic trioxide deposited further along the flue is practically pure white crystalline arsenic trioxide.

In the drawings which illustrate a few forms of apparatus by which the invention may be practiced:

Fig. 1 is a longitudinal section through a refining furnace and the flue thereof which may be used to practice the invention, the flue being modified for practicing the invention;

Fig. 2 is an enlarged longitudinal section through the flue showing the construction of the baffles for the deposition of the vitreous arsenic trioxide, this section being taken on the line 2-2 of Fig. 3;

Fig. 3 is a section taken on the line 3-3 of Fig. 2 showing the baffle construction;

Fig. 4 is a longitudinal section through the flue showing the construction of a modified form of baffle; and

Fig. 5 is a section taken along the line 5-5 of Fig. 4.

Referring now to the drawing and more particularly to Figs. 1, 2 and 3, the refining furnace may be a reverberatory furnace of any desired construction having a hearth on which the charge of black dust or crude arsenic trioxide may be placed, and a fire box for supplying the necessary heat to run the furnace. The fire box may have a charge

door 2 in the wall thereof for introducing fuel therein. Through the roof of the furnace over the hearth may be a charging port through which the charges of crude arsenic trioxide may be introduced.

Preferably spaced from the refining furnace proper is a flue which may be generally rectangular in cross section and which may be divided into two sections. The first section is the baffle section or the section for the deposition of the vitreous oxide of arsenic, and further along the flue is the section for the deposition of pure crystalline oxide of arsenic and which is free from baffles, this section being commonly known as the "kitchen." The flue is connected to the furnace by a connecting pipe or flue 3 which may be of any construction. The connecting pipe and checker work or baffle section of the flue may be covered with a suitable layer of heat insulation 4 to control the temperature of the fumes in the flue.

In one form of apparatus for practicing the invention the baffle section may comprise series of baffles each series comprising parallel elongated members 5 extending across the flue, the members in alternate series being at right angles to each other. Fig. 3 shows two series of horizontal members and a series of vertical members therebetween. These series may, however, be extended to include any number of alternate rows of baffle plates desired. There should be a suitable number of baffles to provide sufficient area on which the vitreous oxide of arsenic may be deposited and without disturbing the flow of gases too greatly.

Referring now to Figs. 4 and 5, an alternate baffle construction may be provided which may comprise series of short tubes 6 whose axes are parallel to the longitudinal axis of the flue, the tubes in each series being piled one upon the other, as shown. The tubes of alternate series may be slightly offset to insure a good baffle action.

It will be understood that the total surface of the baffles which is available for deposition of the vitreous oxide of arsenic will be controlled by the particular circumstances of the case, such as the character of crude arsenic trioxide, the kind of furnace, and the manner in which it is run, as well as the excellency of the desired product.

In operation, the temperature of the baffle section or condensing portion of the flue near

the refining furnace is carefully regulated to be at a point slightly above the melting point of arsenic trioxide, so that the arsenic trioxide which is condensed in this portion 5 of the flue will be in the form of vitreous oxide of arsenic. The exact temperature will vary with conditions, but a temperature of 350° C. has been found suitable in practice.

The temperature may be controlled by the 10 amount of insulation about the connecting pipe and flue, and also by the temperature at which the furnace is operated which of course will depend on the rate at which the fuel is burned. The amount of air passing through 15 the furnace and flue also may be used for controlling the temperature and is a very important factor for proper operation of the process. The temperature may also be controlled, if desired, by providing special 20 external heating means at the section for the deposition of vitreous oxide of arsenic.

The best results have been obtained by maintaining the amount of air flowing through the refining furnace and flue at the 25 minimum necessary to support combustion of the fuel and also keep the furnace at a temperature sufficient to volatilize arsenic trioxide at a commercially practicable rate. The volume of air is controlled by regulating the 30 draft in the flue system and by taking special precautions to have the furnace and flue tight against the ingress of air except as may be necessary to admit air through the charging door for introducing and burning the fuel.

35 Another reason why the volume of air must be kept low is to allow a comparatively slow cooling of the vapors from the refining furnace as they pass through the flue in order to allow sufficient proportion of the arsenic trioxide vapors to deposit on the baffles in the form of vitreous oxide of arsenic. Furthermore, the antimony present which may be in 40 the form of antimony oxide and which is suspended in the vapor either in the form of 45 vapors or as condensed solid particles, must be in contact with the vitreous oxide of arsenic a sufficient length of time to be absorbed.

It has been found that the antimony content of the refined white arsenic decreases as 50 the surface area of the vitreous oxide of arsenic is increased and as the volume of air flowing through the furnace is decreased.

In practicing the invention under the conditions above pointed out, it has been found 55 that the antimony oxides which are volatilized in the refining furnace are absorbed by the vitreous oxide of arsenic to an extent as high as 30% or more antimony in the vitreous oxide of arsenic. On the other hand the arsenic 60 trioxide vapor which condenses further along the flue in the kitchen has been found to contain very little antimony and is a high grade white arsenic. By practicing the invention it has been found possible to recover 75% to 65 80% of the arsenic trioxide content in crude

arsenic trioxide or black dust containing as high as 6% or more of antimony as high grade white arsenic containing less than 0.7% antimony.

Although a particular method of carrying 70 out my improved process has been fully set forth, it is obvious that various changes may be made in the process or in the separate steps thereof without modifying or changing the essential features and characteristics of the 75 product produced and that such product remains substantially the same although slight modifications may be made in its appearance, texture and in its physical and chemical characteristics. 80

It will be understood that the apparatus disclosed may be changed and that other apparatus may be used to practice the invention.

Although I have shown and described and 85 have pointed out in the annexed claims certain novel features of the invention, it will be understood that various omissions, substitutions and changes in the several steps of the process and in its operation may be made 90 by those skilled in the art without departing from the spirit of the invention.

Having described my invention, I claim:

1. A process for refining crude arsenic trioxide comprising volatilizing the crude arsenic trioxide and passing the volatilized crude arsenic trioxide over a substance which will absorb impurities from the said crude arsenic trioxide to produce pure white arsenic. 95

2. A process for refining crude arsenic trioxide comprising volatilizing the crude arsenic trioxide and passing the volatilized crude arsenic trioxide over vitreous oxide of arsenic which will absorb impurities from the crude arsenic trioxide to produce pure white 100 arsenic. 105

3. A process for refining crude arsenic trioxide having antimony as an impurity which comprises volatilizing the crude arsenic trioxide at such temperature that part thereof 110 will condense in the form of vitreous oxide of arsenic, allowing the remainder of the volatilized crude arsenic to pass over the vitreous oxide of arsenic, whereby the vitreous oxide of arsenic will absorb the antimony, and condensing the volatilized arsenic as pure white 115 arsenic oxide. 120

4. A process for refining crude arsenic trioxide of high antimony content comprising heating the crude arsenic trioxide in a refining furnace to volatilize the arsenic trioxide, conducting the vapors and gases from the refining furnace through a section of flue for the condensation of vitreous oxide of arsenic, so controlling the temperature of this section 125 of flue and so controlling the volume of air flowing through the furnace and flue as to allow a portion of the arsenic trioxide vapor to condense as vitreous arsenic oxide and to allow a time of contact of the gases and vapors 130

from the refining furnace with the vitreous arsenic oxide ample for the absorption of most of the antimony, and condensing the purified arsenic trioxide vapor as high grade 5 white arsenic in the remaining section of the flue.

5. A process of refining crude arsenic trioxide having antimony as an impurity, which comprises volatilizing the crude arsenic trioxide in a furnace, exposing the fume of crude arsenic trioxide to vitreous arsenic oxide, controlling the air through the furnace so as to allow the fume sufficient time of contact with the vitreous arsenic oxide for the absorption 10 of most of the antimony.

6. A process for removing antimonial com-

pounds from a given substance which comprises exposing the substance to vitreous arsenic oxide.

7. A process for removing antimonial com- 20 pounds from a given substance, which comprises volatilizing the substance and exposing it to vitreous arsenic oxide.

8. A process of separating arsenic trioxide from a mixture with antimony compounds, 25 which comprises causing a part of the arsenic trioxide to absorb the antimony and removing the remaining purified arsenic trioxide.

In testimony whereof I have hereunto set my hand.

CHESTER L. READ.